



US007811949B2

(12) **United States Patent**  
Snowden et al.

(10) **Patent No.:** US 7,811,949 B2  
(45) **Date of Patent:** Oct. 12, 2010

(54) **METHOD OF TREATING NONWOVEN FABRICS WITH NON-IONIC FLUOROPOLYMERS**

(75) Inventors: **Hue Scott Snowden**, Woodstock, GA (US); **Michael D. Powers**, Canton, GA (US); **Phillip Andrew Schorr**, Atlanta, GA (US)

(73) Assignee: **Kimberly-Clark Worldwide, Inc.**, Neenah, WI (US)

(\*) Notice: Subject to any disclaimer, the term of this patent is extended or adjusted under 35 U.S.C. 154(b) by 709 days.

(21) Appl. No.: 10/723,408

(22) Filed: Nov. 25, 2003

(65) **Prior Publication Data**

US 2005/0112970 A1 May 26, 2005

(51) **Int. Cl.**

B32B 5/28 (2006.01)  
B32B 5/26 (2006.01)

(52) **U.S. Cl.** ..... 442/67; 442/65; 442/66; 442/71; 442/79; 442/110; 442/114; 442/381; 442/382

(58) **Field of Classification Search** ..... 442/65, 442/66, 67, 79, 110, 381, 382, 400, 401, 442/71, 114

See application file for complete search history.

(56) **References Cited**

U.S. PATENT DOCUMENTS

|             |         |                  |
|-------------|---------|------------------|
| 2,841,567 A | 7/1958  | Blanton et al.   |
| 3,061,473 A | 10/1962 | Tesoro           |
| 3,338,992 A | 8/1967  | Kinney           |
| 3,341,394 A | 9/1967  | Kinney           |
| 3,502,763 A | 3/1970  | Hartmann         |
| 3,542,615 A | 11/1970 | Dobo et al.      |
| 3,692,618 A | 9/1972  | Dorschner et al. |
| 3,802,817 A | 4/1974  | Matsuki et al.   |

|               |         |                       |
|---------------|---------|-----------------------|
| 3,849,241 A   | 11/1974 | Butin et al.          |
| 3,855,046 A   | 12/1974 | Hansen et al.         |
| 4,000,233 A * | 12/1976 | Gilbert ..... 264/532 |
| 4,041,203 A   | 8/1977  | Brock et al.          |
| 4,115,605 A   | 9/1978  | Hultman et al.        |
| 4,169,062 A * | 9/1979  | Weipert ..... 428/394 |
| 4,340,563 A   | 7/1982  | Appel et al.          |
| 4,365,049 A   | 12/1982 | Tsunoda et al.        |
| 4,382,990 A   | 5/1983  | Coates                |
| 4,411,928 A   | 10/1983 | Baldwin               |

(Continued)

FOREIGN PATENT DOCUMENTS

EP 0160402 B1 7/1991

(Continued)

OTHER PUBLICATIONS

Dictionary definition of "topical" The American Heritage® Dictionary of the English Language, Fourth Edition Copyright © 2000 by Houghton Mifflin Company. (no month).\*

(Continued)

Primary Examiner—Andrew T Piziali

(74) Attorney, Agent, or Firm—Dority & Manning, P.A.

(57)

**ABSTRACT**

The present invention provides a method of treating a non-woven fabric to improve alcohol repellency that includes contacting a nonwoven fabric with an aqueous treatment solution that includes a non-ionic fluoropolymer and essentially no antistatic agent or less than 0.05 weight percent by weight of an antistatic agent. The present invention also provides a nonwoven fabric with improved alcohol repellency.

**12 Claims, 4 Drawing Sheets**



## U.S. PATENT DOCUMENTS

|               |         |                     |                 |         |                  |
|---------------|---------|---------------------|-----------------|---------|------------------|
| 4,426,476 A   | 1/1984  | Chang               | 6,127,485 A     | 10/2000 | Klun et al.      |
| 4,467,013 A   | 8/1984  | Baldwin             | 6,197,378 B1    | 3/2001  | Clark et al.     |
| 4,547,558 A   | 10/1985 | Iwatsuki            | 6,225,403 B1    | 5/2001  | Knowlton         |
| 4,566,981 A   | 1/1986  | Howells             | 6,274,060 B1    | 8/2001  | Sakashita et al. |
| 4,606,737 A   | 8/1986  | Stern               | 6,297,304 B1    | 10/2001 | Raiford et al.   |
| 4,668,726 A   | 5/1987  | Howells             | 6,350,399 B1    | 2/2002  | Cook et al.      |
| 4,721,511 A   | 1/1988  | Kupits              | 6,562,428 B1    | 5/2003  | Ohrui            |
| 4,795,668 A   | 1/1989  | Krueger et al.      | 6,752,840 B1    | 6/2004  | Onishi et al.    |
| 4,806,410 A   | 2/1989  | Armington et al.    | 6,787,184 B2    | 9/2004  | Snowden et al.   |
| 4,818,597 A   | 4/1989  | DaPonte et al.      | 2002/0025749 A1 | 2/2002  | Shimizu et al.   |
| 4,976,741 A   | 12/1990 | Hisamoto et al.     | 2004/0124565 A1 | 7/2004  | Schiffer et al.  |
| 5,023,130 A * | 6/1991  | Simpson et al. .... | 442/408         |         |                  |
| 5,041,304 A   | 8/1991  | Kusano et al.       | EP 0196759 B1   | 8/1992  |                  |
| 5,045,133 A   | 9/1991  | DaPonte et al.      | EP 0 737 773 A1 | 10/1996 |                  |
| 5,057,368 A   | 10/1991 | Largman et al.      | EP 0 985 741 A1 | 3/2000  |                  |
| 5,069,970 A   | 12/1991 | Largman et al.      | EP 1 039 018 A1 | 9/2000  |                  |
| 5,084,306 A   | 1/1992  | McLellan et al.     | EP 0 815 306 B1 | 7/2002  |                  |
| 5,108,820 A   | 4/1992  | Kaneko et al.       | EP 0 624 680 B1 | 10/2002 |                  |
| 5,132,028 A   | 7/1992  | Nagase et al.       | GB 1346098      | 2/1974  |                  |
| 5,145,727 A   | 9/1992  | Potts et al.        | WO WO 94/24179  | 10/1994 |                  |
| 5,149,576 A   | 9/1992  | Potts et al.        | WO WO 97/08243  | 6/1997  |                  |
| 5,151,321 A   | 9/1992  | Reeves et al.       | WO WO 00/52709  | 9/2000  |                  |
| 5,156,780 A   | 10/1992 | Kenigsberg et al.   | WO WO 01/46507  | 6/2001  |                  |
| 5,169,706 A   | 12/1992 | Collier, IV et al.  | WO WO 01/49925  | 7/2001  |                  |
| 5,178,931 A   | 1/1993  | Perkins et al.      | WO WO 02/083406 | 10/2002 |                  |
| 5,178,932 A   | 1/1993  | Perkins et al.      | WO WO 02/103107 | 12/2002 |                  |
| 5,188,885 A   | 2/1993  | Timmons et al.      | WO WO 03/041458 | 5/2003  |                  |
| 5,194,541 A   | 3/1993  | Legros et al.       |                 |         |                  |
| 5,229,465 A   | 7/1993  | Tsuchida et al.     |                 |         |                  |
| 5,277,976 A   | 1/1994  | Hogle et al.        |                 |         |                  |
| 5,296,282 A * | 3/1994  | Evers ....          | 428/195.1       |         |                  |
| 5,336,552 A   | 8/1994  | Strack et al.       |                 |         |                  |
| 5,349,003 A   | 9/1994  | Kato et al.         |                 |         |                  |
| 5,382,400 A   | 1/1995  | Pike et al.         |                 |         |                  |
| 5,411,576 A   | 5/1995  | Jones et al.        |                 |         |                  |
| 5,436,399 A   | 7/1995  | Koyama et al.       |                 |         |                  |
| 5,466,410 A   | 11/1995 | Hills               |                 |         |                  |
| 5,508,343 A   | 4/1996  | Holley              |                 |         |                  |
| 5,520,962 A   | 5/1996  | Jones, Jr.          |                 |         |                  |
| 5,540,992 A   | 7/1996  | Marcher et al.      |                 |         |                  |
| 5,589,258 A   | 12/1996 | Maddern et al.      |                 |         |                  |
| 5,630,846 A   | 5/1997  | Hara et al.         |                 |         |                  |
| 5,711,994 A   | 1/1998  | Powers              |                 |         |                  |
| 5,804,625 A   | 9/1998  | Temperante et al.   |                 |         |                  |
| 5,851,595 A   | 12/1998 | Jones, Jr.          |                 |         |                  |
| 5,885,909 A   | 3/1999  | Rudisill et al.     |                 |         |                  |
| 6,028,132 A   | 2/2000  | Hayashi             |                 |         |                  |
| 6,114,419 A   | 9/2000  | Liss et al.         |                 |         |                  |

## FOREIGN PATENT DOCUMENTS

|    |              |         |
|----|--------------|---------|
| EP | 0196759 B1   | 8/1992  |
| EP | 0 737 773 A1 | 10/1996 |
| EP | 0 985 741 A1 | 3/2000  |
| EP | 1 039 018 A1 | 9/2000  |
| EP | 0 815 306 B1 | 7/2002  |
| EP | 0 624 680 B1 | 10/2002 |
| GB | 1346098      | 2/1974  |
| WO | WO 94/24179  | 10/1994 |
| WO | WO 97/08243  | 6/1997  |
| WO | WO 00/52709  | 9/2000  |
| WO | WO 01/46507  | 6/2001  |
| WO | WO 01/49925  | 7/2001  |
| WO | WO 02/083406 | 10/2002 |
| WO | WO 02/103107 | 12/2002 |
| WO | WO 03/041458 | 5/2003  |

## OTHER PUBLICATIONS

- INDA Standard Test, IST 80.9-74 (R-82), "Alcohol Repellency of Nonwovens", 1974 (R1982), 3 pages.
- INDA Standard Test, IST 40.2-92, "Electrostatic Decay", 1992, pp. 77-82.
- Method 5514, Federal Test Method Standard No. 191A, "Water Resistance of Cloth; Low Range, Hydrostatic Pressure Method", Jul. 1978.
- Method 5450, Federal Test Method Standard No. 191A, "Permeability to Air; Cloth; Calibrated Orifice Method", Jul. 1978.
- ASTM Designation: D 737-96, "Standard Test Method for Air Permeability of Textile Fabrics", Published Apr. 1996, pp. 207-211.
- Abstract, JP 2002-302871 A2, Oct. 18, 2002.
- Abstract, JP 02656807 B2, Sep. 24, 1997.
- Abstract, JP 02981535 B2, Nov. 22, 1999.
- Abstract, JP 03270930 B2, Apr. 2, 2002.
- Database WPI, Derwent Publications Ltd., JP 9143882A, Jun. 3, 1997.
- Patent Abstracts of Japan, JP 08284067A, Oct. 29, 1996.

\* cited by examiner



FIG. 1



FIG. 2



FIG. 3



FIG. 4

**METHOD OF TREATING NONWOVEN  
FABRICS WITH NON-IONIC  
FLUOROPOLYMERS**

TECHNICAL FIELD

This invention relates to nonwoven fabrics and to methods of treating nonwoven fabrics.

BACKGROUND OF THE INVENTION

The manufacture of nonwoven fabrics for diverse applications has become a highly developed technology. Methods of manufacturing nonwoven fabrics include spunbonding, meltblowing, carding, airlaying, and so forth. It is not always possible, however, to produce by these methods a nonwoven fabric having all desired attributes for a given application. As a result, it is often necessary to treat nonwoven fabrics by various means to impart desired properties. For example, for medical applications such as surgeon's gowns, barrier properties to alcohol and blood penetration and bacteria are desired, and antistatic properties are important as well. Unfortunately, treatments for barrier properties using fluorocarbons, for example, and treatments for antistatic properties using salts are detrimental to each other which makes it necessary to apply excessive amounts of one or both of the treatments. Current methods of treating nonwoven fabrics require slightly to moderately charged, either cationic or anionic, fluoropolymers suspended in water and then combined with anionic antistatic agents in a single bath treatment to produce an alcohol repellent, antistatic surgical fabric. Unfortunately, the antistatic agents currently being used are surface active in nature and negatively impact the water repellency of the finished web as measured by hydrostatic head testing. In addition, the antistatic agents tend to destabilize ionic fluoropolymer suspensions, leading to coagulation and filter plugging issues. Efforts to completely remove the antistat from the bath and apply it downstream on the body side of the web have resulted in a loss of alcohol repellency at equivalent fluoropolymer bath concentrations due to low adsorbed amounts of fluoropolymer on the fabric.

Accordingly, there is a need for a method of topically treating surgical fabric with an alcohol repellent chemistry that does not negatively effect the water barrier of the fabric.

SUMMARY OF THE INVENTION

The present invention provides a method of treating nonwoven fabric with an alcohol repellent chemistry. In one embodiment, the method of the present invention includes contacting a substrate with a treatment solution comprising a non-ionic fluoropolymer and water wherein the treatment solution contains no or less than about 0.05 weight percent by weight of an antistatic agent. The nonwoven substrate can be or include a nonwoven fabric laminate, such as a spunbond/meltblown (SM) laminate, a spunbond/meltblown/spunbond (SMS) laminate, a spunbond/film/spunbond (SFS) laminate, a spunbond/film/spunbond/meltblown/spunbond (SFSMS) laminate or a spunbond/film/film/spunbond (SFFS) laminate. Treated fabric laminates of the present invention are useful as surgical fabrics.

In one embodiment, the present invention provides a method of treating a nonwoven fabric to improve the alcohol repellency of the nonwoven fabric while minimizing any negative effect of the treatment on the water repellency of the nonwoven fabric, the method including contacting a nonwoven fabric with an aqueous treatment solution that includes

from about 0.1 weight percent to about 0.9 weight percent of a non-ionic fluoropolymer and essentially no antistatic agent or less than 0.05 weight percent of an antistatic agent, wherein the hydrostatic head value of the treated nonwoven fabric drops by no more than 45 percent relative to the hydrostatic head value of the untreated nonwoven fabric. Desirably, the hydrostatic head value of the treated nonwoven fabric drops by no more than 30 percent relative to the hydrostatic head value of the untreated nonwoven fabric, more desirably by no more than 25 percent, even more desirably by no more than 20 percent, still more desirably by no more than 15 percent and most desirably by no more than 10 percent relative to the hydrostatic head value of the untreated nonwoven fabric. The treatment solution can be an aqueous treatment solution and include dipping or running the nonwoven fabric or a portion of the nonwoven fabric in to a container of the aqueous treatment solution. Desirably, the aqueous treatment solution is a stable dispersion of non-ionic fluoropolymer in water and wherein the hydrostatic head value of the treated nonwoven fabric drops by no more than 25 percent relative to the hydrostatic head value of the untreated nonwoven fabric. The nonwoven fabric can be selected from the group consisting of spunbond fabrics, meltblown fabrics and laminates thereof. Desirably the treatment solution includes less than 0.005 weight percent by weight of an antistatic agent. More desirably, the treatment solution includes no antistatic agent and the method further includes contacting the nonwoven fabric with a second solution that includes an antistatic agent in a later process step. For example, it is suggested that the method further includes contacting one side of the treated nonwoven fabric with a second treatment comprising an antistatic agent to improve antistatic properties. Desirably, the hydrostatic head value of the treated nonwoven fabric drops by no more than 10 percent relative to the hydrostatic head value of the untreated nonwoven fabric. The antistatic agent can be an organic phosphate ester. In at least one embodiment, the present invention provides a treated nonwoven fabric with improved alcohol repellency that has a hydrostatic head value of greater than 45 mBar as measured by Federal Test Standard 191A, Method 5514. More desirably, the present invention provides a treated nonwoven fabric that has an alcohol repellency of at least 70 percent as measured by INDA Standard Test No. IST 80.9-74 (R-82) and a hydrostatic head value of greater than 45 mBar as measured by Federal Test Standard 191A, Method 5514 and the hydrostatic head value of the nonwoven fabric is decreased by less than 10 percent relative to the untreated nonwoven fabric. Still more desirably, the treated nonwoven fabric has an alcohol repellency of at least 75 percent as measured by INDA Standard Test No. IST 80.9-74 (R-82) and a hydrostatic head value of greater than 45 mBar as measured by Federal Test Standard 191A, Method 5514. The nonwoven fabric can be a laminate that includes at least one spunbond layer and more desirably at least one meltblown layer. For example, the nonwoven fabric can be an infection control fabric that is or includes a spunbond/meltblown/spunbond laminate, a spunbond/film/spunbond laminate, a spunbond/film/spunbond/meltblown/spunbond laminate or a spunbond/film/film/spunbond laminate. In some embodiments, the treatment solution includes greater than about 0.15 weight percent of a non-ionic fluoropolymer or a mixture of non-ionic fluoropolymers. In other embodiments, the treatment solution includes greater than about 0.20 weight percent of a non-ionic fluoropolymer or a mixture of non-ionic fluoropolymers. In still other embodiments, the treatment solution includes greater than about 0.25 weight percent of a non-ionic fluoropolymer or a mixture of non-ionic fluoropolymers. The treatment solution may further include an

optional alcohol, for example an alkyl alcohol. The non-ionic fluoropolymer or fluoropolymers can be selected from the group consisting of fluoroalkyl acrylate homopolymers, fluoroalkyl acrylate copolymers, fluorinated siloxanes, fluorinated silicones, fluorinated urethanes, and mixtures thereof. In at least one embodiment, the non-ionic fluoropolymer is a non-ionic fluoroalkyl acrylate copolymer.

The present invention also provides nonwoven fabrics treated according to the methods of the present invention, particularly nonwoven fabrics that are adapted for use as an infection control product. In one desirable embodiment, the nonwoven fabric includes a first surface and a second, opposing surface wherein the first surface includes a non-ionic fluoropolymer and the second surface includes an antistatic agent. The nonwoven fabric can be a laminate or a portion of a laminate.

In still another embodiment, present invention provides a method of improving the alcohol repellency of a nonwoven laminate by applying a topical treatment to a nonwoven laminate while minimizing any negative effect of the topical treatment on the water repellency of the nonwoven laminate, the method including the steps of: providing a nonwoven laminate; contacting an aqueous treatment solution that includes from about 0.20 weight percent to about 5 weight percent of a non-ionic fluoropolymer or a mixture of non-ionic fluoropolymers with the nonwoven laminate or a portion of the nonwoven laminate where the non-ionic fluoropolymers are selected from the group consisting of non-ionic fluoroalkyl acrylate homopolymers, fluoroalkyl acrylate copolymers, fluorinated siloxanes, fluorinated silicones, fluorinated urethanes, and mixtures thereof; and then contacting a surface of the topically treated nonwoven laminate with an antistatic agent selected from the group consisting of organic phosphate esters.

#### BRIEF DESCRIPTION OF THE DRAWINGS

The invention will be more fully understood and further advantages will become apparent when reference is made to various embodiments described in the following description and accompanying drawings in which:

FIG. 1 is a schematic of one treatment process embodiment of the present invention using a saturation treatment step followed by a spray treatment step.

FIG. 2 is a schematic of a second treatment process embodiment of the present invention using a foam applicator instead of a spray treatment step.

FIG. 3 is a schematic of an exemplary second step of a process of the invention using ink jet treating.

FIG. 4 is a schematic of a third treatment embodiment of the present invention applying antistat and repellent treatments to opposite sides.

Repeated use of reference characters in the present specification and drawings is intended to represent same or analogous features or elements of the present invention.

#### Test Procedures

Hydrostatic Head: A measure of the liquid barrier properties of a fabric is the hydrostatic head test. The hydrostatic head test determines the height of water (in centimeters) which the fabric will support before a predetermined amount of liquid passes through. A fabric with a higher hydrostatic head reading indicates it has a greater barrier to liquid penetration than a fabric with a lower hydrostatic head. The hydrostatic head test is performed according to Federal Test Standard 191A, Method 5514.

The test is modified to include a screen support of standard synthetic fiber window screen material. The test head of a Textest FX-300 Hydrostatic Head Tester, available from Schmid Corporation, having offices in Spartanburg, S.C. was filled with purified water. The purified water was maintained at a temperature between 65° F. and 85° F. (between about 18.3° C. and 29.4° C.), which was within the range of normal ambient conditions (about 73° F. (about 23° C.) and about 50% relative humidity) at which this test was conducted. An 10 8 inch by 8 inch (about 20.3 cm by 20.3 cm) square sample of the test material was placed such that the test head reservoir was covered completely. The sample was subjected to a standardized water pressure, increased at a constant rate until leakage was observed on the outer surface of the sample material. Hydrostatic pressure resistance was measured at the first sign of leakage in three separate areas of the sample. This 15 test was repeated for forty specimens of each sample material. The hydrostatic pressure resistance results for each specimen were averaged and recorded in millibars. Again, a higher 20 value indicates greater resistance to water penetration and is desirable for barrier applications.

Alcohol: The alcohol repellency test is designed to measure the resistance of nonwoven fabrics to penetration by low surface tension liquids, such as alcohol/water solutions. Alcohol repellency was tested according to the test procedure 25 described as follows. In this test, a fabric's resistance to penetration by low surface energy fluids is determined by placing 0.1 ml of a specified volume percentage of isopropyl alcohol (IPA) solution in several different locations on the 30 surface of the fabric and leaving the specimen undisturbed for 5 minutes. In this test, 0.1 ml of serially diluted isopropyl alcohol and distilled water solutions, ranging from 60 volume percent to 100 volume percent in increments of 10 percent, are placed on a fabric sample arranged on a flat surface. After 35 5 minutes, the surface is visually inspected and the highest concentration retained by the fabric sample is noted. For example, if the minimum value is a 70% IPA solution, i.e. a 40 70% IPA solution is retained by the fabric but an 80% solution penetrates through the fabric to the underlying surface. The 45 grading scale ranges from 0 to 5, with 0 indicating the IPA solution wets the fabric and 5 indicating maximum repellency. Unless stated otherwise, the percent alcohol (IPA) repellency reported indicates the maximum volume percent of IPA that could be added to water while still retaining a 5 rating on the scale at all points of the fabric tested. This procedure is a modification of INDA Standard Test No. IST 80.9-74 (R-82).

Resistance to Blood Penetration (RBP): The blood strikethrough or resistance to blood penetration of a fabric is 50 a measure of the amount of blood which penetrates the fabric at a particular pressure. The blood strikethrough is performed by weighing a blotter placed next to the fabric before and after the test which consists of applying 1 pound per square inch gauge (psig) pressure to the side of the fabric away from the 55 blotter, which side has blood thereon. The pressure is ramped up over approximately 10 seconds and removed when it reaches 1 psig. The difference in the weight of the blotter before and after the test in grams represents the amount of blood which has penetrated the fabric.

Grab Tensile test: The grab tensile test is a measure of 60 breaking strength and elongation or strain of a fabric when subjected to unidirectional stress. This test is known in the art and conforms to the specifications of Method 5100 of the Federal Test Methods Standard 191A. The results are 65 expressed in pounds or grams to break and percent stretch before breakage. Higher numbers indicate a stronger, more stretchable fabric. The term "load" means the maximum load

or force, expressed in units of weight, required to break or rupture the specimen in a tensile test. The term "total energy" means the total energy under a load versus elongation curve as expressed in weight-length units. The term "elongation" means the increase in length of a specimen during a tensile test. The grab tensile test uses two clamps, each having two jaws with each jaw having a facing in contact with the sample. The clamps hold the material in the same plane, usually vertically, separated by 3 inches (76 mm) and move apart at a specified rate of extension. Values for grab tensile strength and grab elongation are obtained using a sample size of 4 inches (102 mm) by 6 inches (152 mm), with a jaw facing size of 1 inch (25 mm) by 1 inch, and a constant rate of extension of 300 mm/min. The sample is wider than the clamp jaws to give results representative of effective strength of fibers in the clamped width combined with additional strength contributed by adjacent fibers in the fabric. The specimen is clamped in, for example, a Sintech 2 tester, available from the Sintech Corporation, 1001 Sheldon Drive, Cary, N.C. 27513, an Instron Model™, available from the Instron Corporation, 2500 Washington Street, Canton, Mass. 02021, or a Thwing-Albert Model INTELLECT II available from the Thwing-Albert Instrument Co., 10960 Dutton Road, Philadelphia, Pa. 19154. This closely simulates fabric stress conditions in actual use. Results are reported as an average of three specimens and may be performed with the specimen in the cross direction (CD) or the machine direction (MD).

Antistatic properties were measured according to INDA Standard Test 40.2-92.

Porosity results were obtained by Frazier Porosity tests, ASTM Standard D737 "Air Permeability of Textile Fabrics," also Method 5450 Federal Test Methods Standard No. 191A, except that the specimen size is 8 inches by 8 inches.

#### Definitions

As used herein and in the claims, the term "comprising" is inclusive or open-ended and does not exclude additional unrecited elements, compositional components, or method steps.

As used herein, the term "nonwoven fabric or web" means a web having a structure of individual fibers or threads which are interlaid, but not in an identifiable manner as in a knitted fabric. Nonwoven fabrics or webs have been formed from many processes such as for example, meltblowing processes, spunbonding processes, and bonded carded web processes. The basis weight of nonwoven fabrics is usually expressed in ounces of material per square yard (osy) or grams per square meter (gsm) and the fiber diameters useful are usually expressed in microns or an equivalent but more recognized term, micrometers. (Note that to convert from osy to gsm, multiply osy by 33.91). As used herein the term "spunbonded fibers" refers to small diameter fibers which are formed by extruding molten thermoplastic material as filaments from a plurality of fine, usually circular capillaries of a spinneret with the diameter of the extruded filaments then being rapidly reduced as by, for example, in U.S. Pat. No. 4,340,563 to Appel et al., U.S. Pat. No. 3,692,618 to Dorschner et al., U.S. Pat. No. 3,802,817 to Matsuki et al., U.S. Pat. Nos. 3,338,992 and 3,341,394 to Kinney, U.S. Pat. No. 3,502,763 to Hartman, and U.S. Pat. No. 3,542,615 to Dobo et al. Spunbond fibers are generally not tacky when they are deposited onto a collecting surface. Spunbond fibers are generally continuous and have average diameters (from a sample of at least 10) larger than 7 microns, more particularly, between about 10 and 20 microns. The fibers may also have shapes such as those described in U.S. Pat. No. 5,277,976 to Hogle et al., U.S. Pat.

No. 5,466,410 to Hills and U.S. Pat. Nos. 5,069,970 and 5,057,368 to Largman et al., which describe fibers with unconventional shapes.

As used herein, the term "meltblown fibers" means fibers formed by extruding a molten thermoplastic material through a plurality of fine, usually circular, die capillaries as molten threads or filaments into converging high velocity, usually hot, gas (e.g. air) streams which attenuate the filaments of molten thermoplastic material to reduce their diameter, which 10 may be to microfiber diameter. Thereafter, the meltblown fibers are carried by the high velocity gas stream and are deposited on a collecting surface to form a web of randomly dispersed meltblown fibers. Such a process is disclosed, for example, in U.S. Pat. No. 3,849,241 to Butin et al. Meltblown 15 fibers are microfibers which may be continuous or discontinuous, are generally smaller than 10 microns in average diameter, and are generally tacky when deposited onto a collecting surface.

As used herein, the term "multilayer laminate" means a 20 laminate wherein some of the layers, for example, are spunbond and some meltblown such as a spunbond/meltblown/spunbond (SMS) laminate and others as disclosed in U.S. Pat. No. 4,041,203 to Brock et al., U.S. Pat. No. 5,169,706 to Collier, et al., U.S. Pat. No. 5,145,727 to Potts et al., U.S. Pat. 25 No. 5,178,931 to Perkins et al. and U.S. Pat. No. 5,188,885 to Timmons et al. Such a laminate may be made by sequentially depositing onto a moving forming belt first a spunbond fabric layer, then a meltblown fabric layer and last another spunbond layer and then bonding the laminate in a manner 30 described below. Alternatively, the fabric layers may be made individually, collected in rolls, and combined in a separate bonding step. Such fabrics usually have a basis weight of from about 0.1 to 12 osy (3 to 400 gsm), or more particularly from about 0.75 to about 3 osy. Multilayer laminates may also 35 have various numbers of meltblown layers or multiple spunbond layers in many different configurations and may include other materials like films (F) or coform materials, e.g. SMMS, SM, SFS, etc.

As used herein, the term "polymer" generally includes but 40 is not limited to, homopolymers, copolymers, such as for example, block, graft, random and alternating copolymers, terpolymers, etc. and blends and modifications thereof. Furthermore, unless otherwise specifically limited, the term "polymer" shall include all possible geometrical configurations 45 of the molecule. These configurations include, but are not limited to isotactic, syndiotactic and random symmetries.

As used herein, the term "conjugate fibers" refers to fibers 50 which have been formed from at least two polymers extruded from separate extruders but spun together to form one fiber. Conjugate fibers are also sometimes referred to as multicomponent or bicomponent fibers. The polymers are usually different from each other though conjugate fibers may be monocomponent fibers. The polymers are arranged in substantially 55 constantly positioned distinct zones across the cross-section of the conjugate fibers and extend continuously along the length of the conjugate fibers. The configuration of such a conjugate fiber may be, for example, a sheath/core arrangement wherein one polymer is surrounded by another or may be a side by side arrangement, a pie arrangement or an 60 "islands-in-the-sea" arrangement. Conjugate fibers are taught in U.S. Pat. No. 5,108,820 to Kaneko et al., U.S. Pat. No. 4,795,668 to Krueger et al., U.S. Pat. No. 5,540,992 to Marcher et al. and U.S. Pat. No. 5,336,552 to Strack et al. Conjugate fibers are also taught in U.S. Pat. No. 5,382,400 to 65 Pike et al. and may be used to produce crimp in the fibers by using the differential rates of expansion and contraction of the two (or more) polymers. Crimped fibers may also be pro-

duced by mechanical means and by the process of German Patent no. DT 25 13 251 A1. For two component fibers, the polymers may be present in ratios of 75/25, 50/50, 25/75 or any other desired ratios. The fibers may also have shapes such as those described in U.S. Pat. Nos. 5,277,976 to Hogle et al., U.S. Pat. No. 5,466,410 to Hills and U.S. Pat. Nos. 5,069,970 and 5,057,368 to Largman et al., which describe fibers with unconventional shapes.

As used herein, "thermal point bonding" involves passing a fabric or web of fibers to be bonded between a heated calender roll and an anvil roll. The calender roll is usually, though not always, patterned in some way so that the entire fabric is not bonded across its entire surface, and the anvil roll is usually flat. As a result, various patterns for calender rolls have been developed for functional as well as aesthetic reasons. One example of a pattern has points and is the Hansen Pennings or "H&P" pattern with about a 30% bond area with about 200 bonds/square inch as taught in U.S. Pat. No. 3,855,046 to Hansen and Pennings. The H&P pattern has square point or pin bonding areas wherein each pin has a side dimension of 0.038 inches (0.965 mm), a spacing of 0.070 inches (1.778 mm) between pins, and a depth of bonding of 0.023 inches (0.584 mm). The resulting pattern has a bonded area of about 29.5%. Another typical point bonding pattern is the expanded Hansen Pennings or "EHP" bond pattern which produces a 15% bond area with a square pin having a side dimension of 0.037 inches (0.94 mm), a pin spacing of 0.097 inches (2.464 mm) and a depth of 0.039 inches (0.991 mm). Another typical point bonding pattern designated "714" has square pin bonding areas wherein each pin has a side dimension of 0.023 inches, a spacing of 0.062 inches (1.575 mm) between pins, and a depth of bonding of 0.033 inches (0.838 mm). The resulting pattern has a bonded area of about 15%. Yet another common pattern is the C-Star pattern which has a bond area of about 16.9%. The C-Star pattern has a cross-directional bar or "corduroy" design interrupted by shooting stars. Other common patterns include a diamond pattern with repeating and slightly offset diamonds with about a 16% bond area and a wire weave pattern looking as the name suggests, e.g. like a window screen, with about a 19% bond area. Typically, the percent bonding area varies from around 10% to around 30% of the area of the fabric laminate web. As is well known in the art, the spot bonding holds the laminate layers together as well as imparts integrity to each individual layer by bonding filaments and/or fibers within each layer.

As used herein, the term "infection control product" means medically oriented items such as surgical gowns and drapes, face masks, head coverings like bouffant caps, surgical caps and hoods, footwear like shoe coverings, boot covers and slippers, wound dressings, bandages, sterilization wraps, wipers, garments like lab coats, coveralls, aprons and jackets, patient bedding, stretcher and bassinet sheets, and the like.

As used herein the term "antistatic agent" refers to a reagent capable of preventing, reducing or dissipating static electrical charges that may be produced on textile materials such as nonwoven surgical gowns. Antistatic agents include ZELEC® organic phosphate esters available from Stepan Chemical and QUADRASTAT® mono- and di-substituted potassium isobutyl phosphate from Manufacturers Chemical of Cleveland, Tenn.

Composition percent amounts herein are expressed by weight unless otherwise indicated.

#### DETAILED DESCRIPTION OF THE INVENTION

The present invention relates to treatment of nonwoven substrates to impart desired properties, particularly alcohol

repellency, to the nonwoven substrates. Suggested nonwoven substrates include, but are not limited to, nonwoven fabrics including laminates that include at least one meltblown (M) layer and/or at least one spunbond layer (S), spunbond/meltblown (SM) laminates, spunbond/meltblown/spunbond (SMS) laminates, spunbond/film/spunbond (SFS) laminates, spunbond/film/spunbond/meltblown/spunbond (SFSMS) laminates and spunbond/film/film/spunbond (SFFS) laminate and laminates and combinations thereof. The invention 10 also relates to resulting nonwoven fabrics having, for example, one surface that is alcohol repellent and the other that has antistatic properties suitable for use in the manufacture of infection control medical products including surgical gowns and sterilization wrap. Such nonwoven fabrics also 15 have excellent barrier properties as measured by hydrostatic head and are useful as surgical fabrics and as components in surgical gowns, drapes, surgical packs and so forth. Advantageously, fabrics and fabric laminates of the present invention 20 can be made at lower basis weights while maintaining acceptable barrier properties.

The present invention is described by reference to the test methods and definitions described above and to specific embodiments of the invention, one or more examples of which are set forth below. Each example is provided by way 25 of explanation of the invention, not as a limitation of the invention. In fact, it will be apparent to those skilled in the art that various modifications and variations can be made in this invention without departing from the scope or spirit of the invention. For instance, features illustrated or described as 30 part of one embodiment can be used on another embodiment to yield a still further embodiment. Thus, it is intended that the present invention cover such modifications and variations as come within the scope of the appended claims and their equivalents. Other objects, features and aspects of the present 35 invention are disclosed in or are obvious from the following detailed description. It is to be understood by one of ordinary skill in the art that the present discussion is a description of exemplary embodiments only, and is not intended as limiting the broader aspects of the present invention, which broader 40 aspects are embodied in the exemplary constructions.

The present invention provides an improved method of 45 topically treating nonwoven fabrics with a fluoropolymer chemistry that improves the alcohol repellency of the fabric while minimizing any negative effect on the water barrier of the fabric. In one exemplary embodiment, the method of 50 treating nonwoven fabrics includes treating a nonwoven fabric with a solution or a suspension that includes a non-ionic fluoropolymer, no antistatic agent or essentially no antistatic agent. It is believed that inclusion of antistatic agents negatively 55 effect the water repellency of the fabric. Desirably, the amount of antistatic agent in the treatment solution is less than 0.05 weight percent, even more desirably, less than 0.005 weight percent. Antistatic agents have been observed to destabilize ionic fluoropolymer suspensions of charged fluoropolymers in the treatment bath solution or suspension. Destabilization of the treatment bath is undesirable and causes coagulation and filter plugging during the treatment 60 process. In one desirable embodiment, the present invention provides a method of topically treating surgical fabric that includes treating the fabric with a solution or suspension that 65 includes a non-ionic fluoropolymer. Non-ionic fluoropolymers include, but are not limited to, non-ionic fluoroalkyl acrylate homopolymers and copolymers, such as fluorinated siloxanes, fluorinated silicones, fluorinated urethanes and so forth. A non-ionic fluoropolymer was obtained from Daikin America, Inc. of Orangeberg, N.Y. an affiliate of Daikin Industries, Ltd of Japan, under the trade designations UNI-

DYNE® S-1072 and UNIDYNE® TG-KC02. UNIDYNE® TG KC-O2 is a non-ionic fluoroalkyl acrylate copolymer emulsion that consists essentially of about 30 to 31 weight percent of a non-ionic fluoroalkyl acrylate copolymer, about 60 to 62 weight percent of water and about 8 weight percent of tripropylene glycol. Another non-ionic fluoropolymer that is commercially available from Mitsubishi International Corporation of New York is REPEARL F-7105. REPEARL F-7105 is an emulsion of about 30 weight percent of a non-ionic fluoroacrylate copolymer, about 60 weight percent of water and about 10 weight percent of dipropylene glycol. It is suggested that the treatment solution or suspension that includes the non-ionic fluoropolymer include no or essentially no anionic antistatic agent. An antistatic agent, anionic or otherwise, can be applied to the treated fabric after the water repellency treatment and on only one side so as to minimize negative effects on water repellency. It is believed that using a non-ionic fluoropolymer treatment rather than an ionic fluoropolymer treatment reduces electrostatic interactions in the treatment solution or suspension and improves bath stability. It is also believed that electrostatic interactions hinder adsorption of the treatment solution onto the fabric.

Antistatic agents are reagents that prevent or greatly reduce electrical charges that may be produced on textile materials and are also referred to as antistats. Antistatic agents include organic phosphate esters such as ZELEC KC, an alkyl phosphate ester from Stepan Chemical that may include mono- and disubstituted potassium n-butyl phosphate and QUADR-ASTAT PIBK, mono- and di-substituted potassium isobutyl phosphate from Manufacturers Chemical of Cleveland, Tenn.

Turning to the drawings, FIG. 1 shows a web 10, for example a nonwoven fabric web, traveling from right to left. At saturation spray device 12, a fluorocarbon spray is applied to both sides. Squeeze nip rolls 14 remove excess fluorocarbon and vacuum extractor 16 removes additional treatment composition as web 10 travels over guide rolls 18. At treatment station 20 an antistat is applied to one side only of web 10 by spray device 22 and at a point preferably prior to full curing of the fluorocarbon. Web 10 is then dried by contact with steam cans 24. It is suggested that only one side, the body side, of a nonwoven fabric that is to be used as a surgical gown or other barrier is treated with an antistat so that the antistat does not interfere with the water repellency of the exterior side of the fabric.

FIG. 2 shows a process using a foam applicator to apply the fluorochemical instead of an antistatic spray device 22 as in FIG. 1. For FIG. 2, the system may be the same as FIG. 1 prior to the antistat spray 20 (FIG. 1) and is not shown. In FIG. 2, foam applicator 32 applies fluorocarbon composition as a foam. Excess is removed in the nip 34 between squeeze rolls 36, and web 10 is directed over steam cans 24 for drying as in FIG. 1.

FIG. 3 shows schematically an exemplary second inline treatment step applied to web 40 having been previously treated as, for example, using the saturation spray device 12 of FIG. 1. In this embodiment, web 40 is unwound from roll 42 and directed around guide roll 44 through printing station 46 including ink jet printhead 48 and web support platen/exhaust hood 50. The web has applied to the surface facing the printhead a light application of the antistat. The web may then be directed by one or more drive rolls 52 and rewound into treated roll 54 or, optionally, otherwise processed.

FIG. 4 shows a third embodiment where the foam applicator 32 is used to apply fluorocarbon to one side of web 10 and spray 22 to apply antistat to the opposite side at steam can 24. Otherwise the process is like the process schematically illustrated in FIG. 2.

## EXAMPLES

The present invention is further described by the examples which follow. Such examples, however, are not to be construed as limiting in any way either the spirit or the scope of the present invention.

For those examples using SMS fabric, the general process for forming the fabric and treating it was as follows:

A spunbond/meltblown/spunbond (SMS) laminate consisting of about 35 weight percent of a first spunbond layer, about 30 weight percent of meltblown layer and about 35 weight percent of a second spunbond layer was formed as described in U.S. Pat. No. 4,041,203 to Brock et al. After forming, the SMS laminate was thermally bonded with a bonding roll resulting in about 15 percent bond area in a wire weave pattern. The fabrics produced for the examples had a basis weight of about 1.5 oz/yd<sup>2</sup> (51 gsm) or a basis weight of about 1 oz/yd<sup>2</sup> (about 41 gsm) as specified. After bonding, the SMS laminate was treated off line. Samples of the SMS laminate were treated by immersing a sample of the SMS laminate in a treatment solution as specified below. However, the SMS laminate can be treated in line, for example by passing the SMS laminate through a saturator containing a treatment bath as generally illustrated in FIG. 1. The amount of non-ionic fluoropolymer emulsion needed in the treatment composition is dependent upon the level of alcohol repellency desired and generally believed to be dependent of the specific non-ionic fluoropolymer chosen and the exposure time of the substrate to the treatment composition. In general, the less time that a laminate is exposed to a treatment composition, the greater the amount of non-ionic fluoropolymer emulsion is suggested in the bath to obtain the level of fluorine on the substrate to achieve a targeted level of repellency. Each of the examples was prepared in the same manner. Samples of dried, treated material of each example were tested for alcohol repellency, water barrier as measured by hydrostatic head and fluorine add-on level to determine the add-on efficiency of the method.

The treatment compositions varied as specified in the each 40 of the following Examples. A fluorine containing compound, for example a non-ionic fluoropolymer, was added to increase the isopropanol repellency of the finished, dried laminate. An alcohol, for example octanol, was added to aid in wetting out the laminate completely. As the water is dried off the laminate 45 in a later step, the alcohol is volatilized. The amount of octanol used was typically 0.25 percent by weight in the aqueous treatment bath. For example in a commercial inline process, after saturation, which results in about 300 percent wet pickup based on fabric weight, the fabric can be run through a squeeze nip, resulting in a reduction in the wet pickup to about 100 percent and then over a dewatering vacuum apparatus, further reducing the wet pickup to about 50 40 percent. After drying using steam cans, the treated fabric can be wound on cardboard cores.

No antistatic agent was applied to the Examples. However, an antistatic agent could be included in the treatment bath or added at as a later treatment step. For example, an organic phosphate ester antistatic agent could be applied to one or both surfaces of the fabric via an atomized spray apparatus. The amount of fluoropolymer emulsion included in the treatment composition can vary and is dependent on several factors including, but not limited to, the level of alcohol repellency desired and the time the substrate is exposed to the treatment solution. In general, the less time that the laminate 55 is exposed to the fluoropolymer containing treatment the more fluoropolymer is needed to reach a targeted level of repellency. For the Daikin UNIDYNE® TG-KC02 non-ionic

## 11

fluoropolymer suspension and the process conditions chosen in the Examples below, treatment compositions containing from about 0.1 to about 1 weight percent of the non-ionic fluoropolymer suspension were used. The amount of fluoropolymer is also believed to be dependent on the particular fluoropolymer that is selected.

The treatment solutions for each example were prepared as follows. The specified weight of fluoropolymer emulsion was added to water in a 1000 ml beaker. The non-ionic fluoropolymer emulsion was initially mixed into the water using a spatula and then placed under a Ross high shear mixer. Under vigorous mixing, the specified amount of other ingredients, if any, and the specified amount of octanol was added to the mixture and further mixed a high speed for an additional 2 minutes. The emulsion was then transferred to a pan large enough to accommodate an 8-inch by 10-inch sample of the SMS fabric. An 8-inch by 10-inch sample of the SMS fabric was then completely submerged in the emulsion and flipped over and submerged in the emulsion again to ensure complete wet out. The saturated SMS fabric was then run through an Atlas laboratory ringer equipped with 100 lbs equivalent weights to reduce the wet pick up (WPU). The resulting emulsion was then fed into a saturation pan and continuously added to maintain the required amount of fluid necessary to saturate the SMS web passing through the equipment. The resulting wet pick up (WPU) of the formulation on the SMS was 300 percent by weight of the SMS. The WPU can be calculated as  $WPU = 100\% \times (\text{wet weight} - \text{dry weight}) / \text{dry weight}$ . The SMS web then passed through a wringer capable of reducing the wet pick up from 300 percent down to 100 percent. The liquid that was removed from the sheet was allowed to recirculate back into the saturation pan. Finally, the treated SMS web passed through a large forced hot air drying unit capable of reducing the WPU from 100 percent to bone dry (0 percent WPU).

The percent fluorine add-on level on the samples was determined by an independent laboratory (Galbraith Laboratories of Knoxville, Tenn.) using an elemental analysis technique. The hydrostatic head of the samples was measured according to Federal Test Standard 191A, Method 5514. The alcohol repellency of the samples was measured by placing 0.1 ml of a specified percentage of isopropyl alcohol aqueous solution in several different locations on the surface of the fabric and leaving the specimen undisturbed for 5 minutes. The grading scale ranges from 0 to 5, with 0 indicating the IPA solution wets the fabric and 5 indicating maximum repellency. Unless stated otherwise, the percent alcohol (IPA) repellency reported indicates the maximum volume percent of IPA that could be added to water while still retaining a 5 rating on the scale at all points of the fabric tested. This procedure is a modification of INDA Standard Test No. IST 80.9-74 (R-82).

## Comparative Example A

Comparative Example A consisted of untreated 1.5 osy SMS laminate fabric. The alcohol repellency of Comparative Example A was measured at 20 percent IPA. The water barrier property of Comparative Example A was measured at a hydrostatic head of  $84.9 \pm 6.2$  mBar. The untreated 1.5 osy SMS fabric provides desirable water barrier but does not provide acceptable alcohol repellency.

## Comparative Example B

Comparative Example B consisted of untreated 1.5 osy SMS laminate fabric that was treated in a bath that included an ionic fluoropolymer and an anionic antistatic agent. The

## 12

aqueous treatment bath for Comparative Example B consisted of water in which was dissolved, or at least suspended, 0.69 weight percent of a cationic fluoropolymer suspension from Daikin America, Inc. identified as UNIDYNE® TG-KC01 and 0.30 weight percent of QUADRASTAT PIBK anionic antistatic agent obtained from Manufacturers Chemical of Cleveland, Tenn. The alcohol repellency of Comparative Example B was measured at 90 percent IPA. The water barrier property of Comparative Example B was measured at a hydrostatic head of  $46.3 \pm 3.1$  mBar. And, the fluorine add-on level of Comparative Example B was measured at 0.36 weight percent.

## Example 1

Example 1 is an example of a dip saturation treatment method of treating a 1.5 osy SMS nonwoven surgical fabric with an aqueous treatment solution that includes a nonionic fluoropolymer and no antistatic agent. The treatment bath suspension of Example 1 consisted of a water bath in which was dissolved, or at least suspended, 0.85 weight percent of a non-ionic fluoropolymer suspension UNIDYNE® TG-KC02 obtained from Daikin America, Inc. of Orangeberg, N.Y. and 0.25 weight percent of octanol (a short chain alcohol that was used as a wetting agent).

The UNIDYNE® TG-KC02 non-ionic fluoropolymer suspension obtained from Daikin contained about 30 weight percent of non-ionic fluoropolymer solids and the wet pick-up rate of the treatment solution on the SMS fabric for Example 1 was about 116 weight percent. The non-ionic fluoropolymer treated SMS surgical fabric was dried for 2 minutes at about 105° C. The alcohol repellency of the dried, non-ionic fluoropolymer treated Example 1 was measured at 60 percent IPA.

## Example 2

The treatment bath suspension of Example 2 consisted of a water bath in which was dissolved, or at least suspended, 1.00 weight percent of UNIDYNE® TG-KC02 non-ionic fluoropolymer suspension obtained from Daikin and 0.25 weight percent of octanol. The wet pick-up rate of the treatment solution on the 1.5 osy SMS fabric for Example 2 was about 116 weight percent. The non-ionic fluoropolymer treated SMS fabric was dried for 2 minutes at about 105° C. The alcohol repellency of the dried, non-ionic fluoropolymer treated Example 2 was measured at 80 percent IPA.

## Comparative Example C

Comparative Example C consisted of untreated 1 osy SMS laminate fabric. The alcohol repellency of Comparative Example A was measured at 20 percent IPA. The water barrier property of Comparative Example A was measured at a hydrostatic head of  $47.3 \pm 5.3$  mBar. The untreated 1 osy SMS fabric provides desirable water barrier but does not provide acceptable alcohol repellency.

## Example 3

The treatment bath suspension of Example 3 consisted of a water bath in which was dissolved, or at least suspended, 0.80 weight percent of UNIDYNE® TG-KC02 non-ionic fluoropolymer suspension obtained from Daikin and 0.25 weight percent of octanol. 1 osy SMS fabric was treated offline after the SMS fabric was produced by running the SMS through the treatment solution at a rate of about 50 feet per minute result-

13

ing in a wet pick-up rate of about 99 weight percent. The wet SMS fabric was then passed through a nip at a pressure of about 50 psi and dried over a drying can at about 245° F. The alcohol repellency of the dried, non-ionic fluoropolymer treated Example 3 was measured at 100 percent IPA. The water barrier property of Example 3 was measured at a hydrostatic head of 47.2±1.5 mBar.

#### Example 4

The treatment bath suspension of Example 4 consisted of a water bath in which was dissolved, or at least suspended, 0.60 weight percent of UNIDYNE® TG-KC02 non-ionic fluoropolymer suspension obtained from Daikin and 0.25 weight percent of octanol. 1 osy SMS fabric was treated offline by running the SMS through the treatment solution at a rate of about 50 feet per minute resulting in a wet pick-up rate of about 99 weight percent. The wet SMS fabric was then passed through a nip at a pressure of about 50 psi and dried over a drying can at about 245° F. The alcohol repellency of the dried, non-ionic fluoropolymer treated Example 4 was measured at 100 percent IPA. The water barrier property of Example 4 was measured at a hydrostatic head of 48.1±3.3 mBar.

#### Example 5

The treatment bath suspension of Example 5 consisted of a water bath in which was dissolved, or at least suspended, 0.40 weight percent of UNIDYNE® TG-KC02 non-ionic fluoropolymer suspension obtained from Daikin and 0.25 weight percent of octanol. 1 osy SMS fabric was treated offline by running the SMS through the treatment solution at a rate of about 50 feet per minute resulting in a wet pick-up rate of about 99 weight percent. The wet SMS fabric was then passed through a nip at a pressure of about 50 psi and dried over a drying can at about 245° F. The alcohol repellency of the dried, non-ionic fluoropolymer treated Example 5 was measured at 95 percent IPA. The water barrier property of Example 5 was measured at a hydrostatic head of 52.4±2.8 mBar.

#### Example 6

The treatment bath suspension of Example 6 consisted of a water bath in which was dissolved, or at least suspended, 0.20 weight percent of UNIDYNE® TG-KC02 non-ionic fluoropolymer suspension obtained from Daikin and 0.25 weight percent of octanol. 1 osy SMS fabric was treated offline by running the SMS through the treatment solution at a rate of about 50 feet per minute resulting in a wet pick-up rate of about 99 weight percent. The wet SMS fabric was then passed through a nip at a pressure of about 50 psi and dried over a drying can at about 245° F. The alcohol repellency of the dried, non-ionic fluoropolymer treated Example 6 was measured at about 80 percent IPA. The water barrier property of Example 6 was measured at a hydrostatic head of 49.3±2.3 mBar.

#### Example 7

The treatment bath suspension of Example 7 consisted of a water bath in which was dissolved, or at least suspended, 0.10 weight percent of UNIDYNE® TG-KC02 non-ionic fluoropolymer suspension obtained from Daikin and 0.25 weight percent of octanol. 1 osy SMS fabric was treated offline by running the SMS through the treatment solution at a rate of

14

about 50 feet per minute resulting in a wet pick-up rate of about 99 weight percent. The wet SMS fabric was then passed through a nip at a pressure of about 50 psi and dried over a drying can at about 245° F. The alcohol repellency of the dried, non-ionic fluoropolymer treated Example 7 was measured at about 40 percent IPA. The water barrier property of Example 7 was measured at a hydrostatic head of 48.3±2.8 mBar.

#### Example 8

The treatment bath suspension of Example 8 consisted of a water bath in which was dissolved, or at least suspended, 1.50 weight percent of a non-ionic fluoropolymer suspension REPEARL F-7105 obtained from Mitsubishi International Corporation of New York and 0.25 weight percent of octanol (a short chain alcohol that was used as a suspending agent) obtained from Aldrich Chemical. The REPEARL F-7105 non-ionic fluoropolymer suspension obtained from Mitsubishi contained about 30 weight percent of non-ionic fluoropolymer solids and the wet pick-up rate of the treatment solution on the 1 osy SMS fabric was about 120 weight percent. The non-ionic fluoropolymer treated 1 osy SMS fabric was dried for 2 minutes at about 105° C. The alcohol repellency of the dried, non-ionic fluoropolymer treated Example 8 was measured at 40 percent IPA.

#### Example 9

The treatment bath suspension of Example 9 consisted of a water bath in which was dissolved, or at least suspended, 2.25 weight percent of REPEARL F-7105 non-ionic fluoropolymer suspension and 0.25 weight percent of octanol. The wet pick-up rate of the treatment solution on the 1 osy SMS fabric for Example 9 was about 90 weight percent. The non-ionic fluoropolymer treated 1 osy SMS fabric was dried for 2 minutes at about 105° C. The alcohol repellency of the dried, non-ionic fluoropolymer treated Example 9 was measured at 50 percent IPA.

A summary of the experimental data is present in Table 1 below.

TABLE 1

| Example Number | Treatment Solution Composition                                             | Isopropyl Alcohol Repellency | Hydrostatic Head (mBar) |
|----------------|----------------------------------------------------------------------------|------------------------------|-------------------------|
| Control A      | untreated 1.5 osy SMS                                                      | 20                           | 84.9 ± 6.2              |
| Control B      | 1.5 osy SMS treated w/<br>0.69 w/o TG-KC01 and<br>0.30 w/o QUADRASTAT PIBK | 90                           | 46.3 ± 3.1              |
| 1              | 1.5 osy SMS treated w/<br>0.85 w/o TG-KC02                                 | 60                           | —                       |
| 2              | 1.5 osy SMS treated w/<br>1.00 w/o TG-KC02                                 | 80                           | —                       |
| Control C      | untreated 1 osy SMS                                                        | 20                           | 47.3 ± 5.3              |
| 3              | 1 osy SMS treated w/<br>0.80 w/o TG-KC02                                   | 100                          | 47.2 ± 1.5              |
| 4              | 1 osy SMS treated w/<br>0.60 w/o TG-KC02                                   | 100                          | 48.1 ± 3.3              |
| 5              | 1 osy SMS treated w/<br>0.40 w/o TG-KC02                                   | 95                           | 52.4 ± 2.8              |
| 6              | 1 osy SMS treated w/<br>0.20 w/o TG-KC02                                   | 80                           | 49.3 ± 2.3              |
| 7              | 1 osy SMS treated w/<br>0.10 w/o TG-KC02                                   | 40                           | 48.3 ± 2.8              |
| 8              | 1 osy SMS treated w/<br>1.50 w/o REPEARL F-7105                            | 40                           | —                       |
| 9              | 1 osy SMS treated w/<br>2.25 w/o REPEARL F-7105                            | 50                           | —                       |

## 15

Although various embodiments of the invention have been described above using specific terms, devices, and methods, such description is for illustrative purposes only. The words used are words of description rather than of limitation. It is to be understood that changes and variations may be made by those of ordinary skill in the art without departing from the spirit or scope of the present invention, which is set forth in the following claims. In addition, it should be understood that aspects of the various embodiments may be interchanged both in whole or in part. Therefore, the spirit and scope of the appended claims should not be limited to the description of the preferred versions contained therein.

We claim:

1. A topically treated nonwoven fabric laminate, the nonwoven fabric laminate comprising at least one spnbond layer and at least one meltblown layer, and the laminate further comprising a dried coating of a non-ionic fluoropolymer composition on said spnbond and meltblown layers, said composition applied in solution form to said laminate so as to permeate and coat all layers of said laminate; and wherein the nonwoven fabric laminate further comprises an antistatic agent applied over said coating of non-ionic fluoropolymer on one side of said laminate, and wherein the antistatic agent is an organic phosphate ester.
2. An infection control product comprising a nonwoven fabric laminate of claim 1.
3. The nonwoven fabric of claim 1 wherein the hydrostatic head value of the treated nonwoven fabric is decreased by no more than 45 percent relative to the hydrostatic head value of an untreated nonwoven fabric.
4. The nonwoven fabric of claim 3 wherein the hydrostatic head value of the treated nonwoven fabric is decreased by no more than 30 percent relative to the hydrostatic head value of an untreated nonwoven fabric.

## 16

5. The nonwoven fabric of claim 4 wherein the hydrostatic head value of the treated nonwoven fabric is decreased by no more than 25 percent relative to the hydrostatic head value of an untreated nonwoven fabric.
6. The nonwoven fabric of claim 5 wherein the hydrostatic head value of the treated nonwoven fabric is decreased by no more than 15 percent relative to the hydrostatic head value of an untreated nonwoven fabric.
7. The nonwoven fabric of claim 1 wherein the nonwoven fabric has a hydrostatic head value of greater than 45 mBar as measured by Federal Test Standard 191A, Method 5514.
- 10 8. The nonwoven fabric of claim 1 wherein the nonwoven fabric has an alcohol repellency of at least 70 percent as measured by INDA Standard Test No. IST 80.9-74 (R-82) and a hydrostatic head value of greater than 45 mBar as measured by Federal Test Standard 191A, Method 5514.
- 15 9. The nonwoven fabric of claim 1 wherein the nonwoven fabric has an alcohol repellency of at least 75 percent as measured by INDA Standard Text No. IST 80.9-74 (R-82) and a hydrostatic head value of greater than 45 mBar as measured by Federal Test Standard 191A, Method 5514.
- 20 10. The nonwoven fabric of claim 1 wherein the nonwoven fabric is an infection control fabric that is or comprises a spnbond/meltblown/spnbond laminate or a spnbond/film/spnbond/meltblown/spnbond laminate.
- 25 11. The nonwoven fabric of claim 1 wherein the non-ionic fluoropolymer is selected from the group consisting of fluoroalkyl acrylate homopolymers, fluoroalkyl acrylate copolymers, fluorinated siloxanes, fluorinated silicones, fluorinated urethanes, and mixtures thereof.
- 30 12. The nonwoven fabric of claim 1 wherein the non-ionic fluoropolymer is a non-ionic fluoroalkyl acrylate copolymer.

\* \* \* \* \*